

Aug. 16, 1932.

H. G. ANDRÉ

1,872,214

RECTIFYING APPARATUS

Original Filed Oct. 1, 1926

Fig. 1



Fig. 3



Fig. 2



Fig. 4



Inventor  
Henri G. André  
By Roberto, Cushman & Woodbury  
Atty's.

## UNITED STATES PATENT OFFICE

HENRI G. ANDRÉ, OF PARIS, FRANCE

## RECTIFYING APPARATUS

Application filed October 1, 1926, Serial No. 138,924. Renewed May 11, 1931.

The present invention relates to electrical apparatus and in particular to alternating current rectifiers in which two metals of different character are employed as electrodes, the metals fulfilling alternately the function of cathode and anode.

In my Patent No. 1,830,500, dated November 3, 1931, of which this is a continuation in part, I have disclosed a rectifier one electrode of which comprises a metallic colloid while the other is formed of a material that when subjected to an oxidizing agent yields a compound which cooperates with the other electrodes to form a unilateral conductor.

In the application identified, I have also stated the presence and manner in which derived of an element in colloidal form making physical contact with one of the electrodes and in particular with the cathode. Apparatus made according to the foregoing specification has the property of rectifying alternating current of comparatively large amplitude.

It has been found in practice that the colloidal element instead of being introduced physically into the space surrounding the cathode, as explained in my application supra, may be formed in place by the action of the current to be rectified, thus eliminating a tedious step in manufacture.

Other changes in construction will be noted in the following description, for example, whereas in the application referred to the cathode is sealed within the surrounding casting by means of sulphur or other amorphous material, manufacturing experience has shown that other methods of securing the cathode are preferable.

The invention described hereinafter has for its purpose a design of rectifier operating on the colloidal principle which offers simplicity of manufacture and ease of operation.

Other features consist in novelty of construction combination and arrangement of parts hereinafter described and claimed, the advantages of which will be obvious to those skilled in the art.

The accompanying drawing illustrates an exemplary embodiment of the device form-

ing the subject of the present invention in which,

Fig. 1 is a vertical section of the improved rectifier;

Fig. 2 is a section taken on line 2—2 of Fig. 1;

Fig. 3 represents a vertical section of another embodiment; while

Fig. 4 shows a section taken on line 4—4 of Fig. 3.

Referring to the illustration, the invention in its preferred form consists of glass tube or envelope 2, the ends of which are closed by stoppers 3, 14 made of rubber or bakelite. The upper stopper has an opening longitudinally of the principal axis of the container for the introduction of fine tube 4 of insulating material, as glass or rubber.

The rectifier proper consists of cathode 13 made preferably of cylindrical form to fit the inner diameter of tube 2 and of a material exhibiting strong electrolytic oxidation, for example aluminum, nickel or one of its alloys, as nickel-silicon, containing 25 to 32% silicon, and nickel-iron. The cathode is in intimate contact with colloidal anode 10 formed in place by electrolytic action occurring in a manner to be described hereinafter. Reference character 8 designates a conductor of material, as silver or graphite, the oxidation compounds of which are good conductors of electrical energy and able to withstand attack by acid, surfacial oxidation excepted. As will be noted from the drawing, electrode 8 is of rectangular cross-section but may also take a cylindrical form and is suspended in the glass envelope by lead wire 5 passing through fine tube 4. The lead wire is preferably of the same metal as the electrode to which it is attached.

For electrolyte 6, which completely submerges electrode 8, I prefer sulfuric acid having concentration of approximately 66° Baumé, although it is to be understood that all fluids capable of producing oxidation of metals, and any degree of concentration comes within the purview of my invention.

In order that the solution may be sufficiently strong to prevent permanent electrolysis and at the same time weak enough to

preserve the electrodes from dissolution by attack, I combine with the acid an anhydrid in approximately 20% proportion, preferably that of phosphoric acid.

- 5 At 7, I have indicated a quantity of glass wool so-called, effectively to hold by absorption acid superfluous or in loose form to the end that the rectifying unit may be handled without spill. Furthermore, the interstices between glass fibres allow passage of the gas evolved during the initial process of electrolysis as will be explained later. The gas may escape to the atmosphere through fine tube 4.
- 10 Cathode 3 is secured within the envelope by filling 14 of rubber poured hot in place, or bakelite, which makes firm contact with the glass wall by baking. A seal in addition to element 14 is provided by layer 15 of plastic compound.

15 The entire rectifying unit is secured preferably in a base of the Edison screw type by plastic material 16 about the periphery of which member 12 makes electrical connection by molybdenum lead 17 with the cathode. It is obvious, however, that under certain conditions a bayonet-slot type of base may be advantageously employed. The base terminates in metallic member 19 to which connection is made from the anode by molybdenum lead 9. For the purpose of protecting the unit from external injury and also to insure convenience of handling, I provide a container or casing 1 of a metal, which 20 shapes conveniently, as lead or brass.

25 This container is open to the atmosphere through apertures 20 and secured to the base by a close fit in metallic annular ring 11. Inasmuch as the principal roles of the enclosing envelope are those of protection and the furnishing of a convenient arrangement for making contact with external circuits, its shape and form may be varied extensively, and I do not intend to limit myself to that 30 shown.

35 The operation of my device is not wholly understood from the theoretical standpoint, but I believe it to be as follows:

40 When alternating current is initially applied to the cathode and anode, electrolytic phenomena take place as evidenced by the evolution of gas in the acid. The silver conductor which initially performs the function of anode appears to disintegrate and in powdered or colloidal form is attracted to the 45 nickel cathode where a relatively thick deposit is formed. This deposit is in the nature of a finely divided mass of metal, each particle of which is partially surrounded by liquid.

50 As indicated on the drawing, the colloid, when examined microscopically, appears to build in a formation resembling the roots of a tree spreading out from the trunk. This 55 action continues until the entire space be-

tween anode and cathode is bridged by colloidal arms of irregular cross-section, having their inception at the silver anode. It is apparent, however, that conditions of operation, as voltage and frequency of the electromotive force applied during the preliminary period, also the size, shape and position of electrodes, each have a marked effect on the manner in which the powdered mass is obtained.

60 As representing another form which the colloid may take, in Fig. 3, I show an electrode arrangement, i. e. cathode uppermost, reversed from the position assumed in Fig. 1. Due in part to gravitational forces, the particles of silver seem to congregate without definite outline between the electrodes, a portion falling to the bottom of the glass envelope. Inasmuch as the latter and the outer metallic shield form no part of the present 65 invention, I will not describe them.

70 Referring to Fig. 4, the section of cathode will be noted as a cross, which shape I have found operates beneficially when the electrodes are in the positions shown.

75 The action just described extends over a short period of time and is a condition precedent to complete rectification of the applied electromotive force, although as a matter of fact I find that partial rectification sets in 80 almost immediately upon application of the alternating potential.

85 At the expiration of the preliminary colloid forming period, electrolytic action appears to cease, and as far as I have been able 90 to determine, the rectifier eventually is devoid of electrolysis. In this specification I intend "electrolysis" to include disintegration of electrodes by an electrolyte either with or without the formation or deformation of 95 a superficial oxide layer. The primary function of the electrolyte, however, is to oxidize the electrodes, which being of dissimilar metal will be affected unequally. In its subsequent 100 operation as a rectifier, the anodal function is 105 transferred to the colloid, electrode 8 assuming the role of a mere conductor or lead.

110 Now I have found that oxidation compounds of nickel and its alloys have the desirable characteristic of permitting current flow 115 in one direction only. This property appears to be utilized to great advantage when operating in conjunction with a colloidal anode that forms many points of physical contact with the adjacent oxide film, offering unilateral 120 conduction of current in aggregate, of a high order.

125 The passage of current from anode to cathode may be explained on the theory of transference of atoms of oxygen direct from the nickel to silver while the insulating property of the nickel oxide film, upon reversal of potential, prevents current passing in the opposite direction. While the silver is also 130 acted upon by an electrolyte, the resulting

compound, oxide of silver, conducts current readily in both directions. Thus the rectifying feature is attributed at present solely to the oxide layer covering the nickelous cathode.

This explanation, however, is offered purely as a matter of interest and which present experience with the rectifier has seemed to dictate.

Whatever are the true principles involved, the fact remains that a rectifier made according to the specification set forth utilizing a nickel-silicon cathode of .093 diameter, a silver anode of .01 square inches cross-section, on test continuously passed rectified direct current of one ampere, delivering a potential of six volts with a loss in the tube of approximately one watt. Such showing, of course, was made after the colloid was formed complete and substantially all electrolytic action had ceased.

While I have illustrated the electrodes relatively close together, it will be appreciated by those skilled in the art, their shape, size and spacing may be varied to meet a specific performance or design. The device disclosed is readily adapted to operate in conjunction with standard circuits utilizing half or full wave rectification. For rectification of both half waves it is obvious that two anodes and a cathode or two cathodes and an anode may be combined for convenience in a single receptacle.

I claim:

1. A unidirectional discharge device having a film-forming electrode and an additional non-film-forming electrode with a mass of finely divided conducting material substantially bridging the space therebetween characterized in that the particle mass comprises a distintegration product of the other electrode and is formed in situ.

2. A unidirectional discharge device comprising a cathode having a unilaterally current conducting layer and a non-film-forming anode associated therewith reduced to subdivided form by the action of the current to be rectified.

3. A unidirectional discharge device comprising in combination, a cathode, the oxidation product of which constitutes a unilateral conductor of current, an anode whose oxide is conducting associated therewith, a member composed of minute particles formed in place and making contact with said cathode and a slightly ionizable liquid to produce oxidation of the latter.

4. In an electrical apparatus, the combination with a non-film-forming anode, of a film forming cathode associated with the said anode and immersed in an electrolyte whereby gas is evolved, and means for absorbing the electrolyte including a fibrous material, the strands of which permit gas flow, the said anode being reducible to par-

ticle form by the action of the current to be rectified.

5. A unidirectional discharge device comprising a cathode having an extended exterior area with a unilaterally conducting layer and a bilaterally conducting anode associated therewith reduced to sub-divided form by passage of current between said anode and said cathode.

6. A unidirectional discharge device comprising a cathode having an extended exterior area with a unilaterally conducting layer and a bilaterally conducting anode in contact with said area reduced to sub-divided form by passage of current between said anode and said cathode.

Signed by me at Boston, Massachusetts, this 17th day of September, 1926.

HENRI G. ANDRÉ